

June 21, 1938.

B. SANFORD

2,121,746

COMPOSITE ABRASIVE WHEEL

Filed Jan. 12, 1937



Fig. 1.



Fig. 2.



Fig. 3.

Witness

Robert G. Trumbull

Inventor

Baalis Sanford

by Clayton L. Jenkins  
Attorney

## UNITED STATES PATENT OFFICE

2,121,746

## COMPOSITE ABRASIVE WHEEL

Baalis Sanford, Worcester, Mass., assignor to  
 Norton Company, Worcester, Mass., a corpora-  
 tion of Massachusetts

Application January 12, 1937, Serial No. 120,275

2 Claims. (Cl. 51—278)

This invention relates to the manufacture of composite grinding wheels and particularly wheels of the type which have a non-abrasive central support carrying a rim of bonded diamonds or 5 other abrasive material.

It has been proposed to make a diamond wheel by pressing a rim of diamond grains and a suitable bond onto a resinoid backing plate which has been previously molded, and thereafter to 10 convert the resinoid to its solid infusible condition by heating the entire wheel structure. Owing to the expense involved as well as the long life of the diamonds, it has been preferred to make the abrasive rim quite narrow. However, 15 in making certain types of wheels, difficulties have been encountered in securing a thin diamond and resinoid rim to a backing plate, due in part to the fact that a thin layer of the plastic resinoid may not flow uniformly and the thickness of 20 the abrasive rim thus varies to an undesired extent.

The primary object of this invention is to overcome such problems and to provide a method of making a composite abrasive wheel of this type 25 and particularly to shape an abrasive rim correctly and secure it firmly to a premolded central support. Other objects will be apparent in the following disclosure.

Referring to the drawing which illustrates two 30 types of wheel molds and a method of shaping wheels therein:

Fig. 1 is a diametrical sectional view showing in a disassembled relationship and distorted sizes a premolded abrasive rim and a premolded back- 35 ing support with a paper cementing strip therebetween which are adapted to be secured together to form a cup shaped wheel;

Fig. 2 is a similar sectional view showing the parts assembled in a mold and ready to be 40 pressed into an integral relationship; and

Fig. 3 is a similar view showing an arrangement of mold and wheel parts for forming a cylindrical wheel support with the abrasive rim secured on the periphery thereof.

In accordance with this invention, an abrasive rim and particularly one made of diamond grains and a resinoid bond or other suitable bonding material, such as vulcanizable rubber, is first premolded to the required shape and dimensions and this ring shaped member is fully cured by means of heat so that the bond is set to a non-plastic and infusible condition. Thereafter, this abrasive ring is secured to a backing support either by a separate cementitious material or by means of plastic flow of the backing

support into an integral union therewith, or by a combination of both features.

Assuming first that a thin flat ring or disk is to be secured onto the side of a grinding wheel, such as the cup shaped rim indicated in Fig. 1, 5 then the following procedure may be adopted. The thin rim 10 of premolded abrasive and a suitable bond, which may be far thinner than indicated in the drawing, is preferably made from a suitable mixture of diamond, boron carbide, silicon carbide, crystalline alumina or other suitable abrasive grains of required grit size and an unconverted resinoid powder, such as a "Bakelite" phenolic formaldehyde condensation product in required proportions, such as 25 to 50 10 parts by weight of diamond grains with the remainder made up of the resinoid bond and suitable fillers, such as silica, wood flour, asbestos, clay or other granular material. This mixture may be placed in a suitable mold and pressed 15 to a required density, and the pressing operation may be either done simultaneously with or followed by a heating operation which sets the resinoid to a solid, non-plastic condition in intimate association with the abrasive grains. The 20 heat setting conditions of temperature and extent of pressure will be in accordance with standard practice. If rubber is employed as the bond 25 then various procedures may be adopted, such as milling a desired quantity of the abrasive 30 grains into a strip of raw rubber compounded with sulfur and a vulcanization accelerator in proportions for making hard rubber. This may be accomplished in accordance with standard 35 methods by repeatedly passing the rubber compound between power driven rollers after folding a quantity of loose abrasive grains into the raw rubber compound. After the rubber and abrasive mixture has been satisfactorily compounded, then the material may be subjected 40 to heat sufficient to vulcanize the rubber to a hard, non-plastic condition.

For the central support 12, which in Fig. 1 is shown as a cup shaped member provided with a central hole, it is preferred that this member be made of a material similar to that of the bond of the abrasive ring 10. That is, a resinoid center is used with a resinoid bonded rim, and a rubber center with a rubber bonded rim. In making a resinoid center, a suitable filler if used 50 and the unconverted resinoid in powdered form, or if desired in a liquid condition, are intermixed and placed in a mold and then shaped under adequate pressure to cause the mass to assume substantially its final density. It is pre- 55

ferred that this resinoid compound be one of low molding shrinkage, that is, having a high percentage of a filler such as flint, wood flour, asbestos and other suitable compounds, so that during the subsequent molding operations the central backing support will retain substantially its original volume. The resinoid of this backing support should preferably remain unconverted to the non-plastic condition so as to make use of that property of plastic flow which the material possesses when subjected to the high pressure of the next step of the molding operation; but it may be converted, if desired, to its final non-plastic condition prior to the step of fastening the premolded abrasive rim thereon.

For a cementing medium to secure the two premolded parts together, I may employ a "Bakelite" resinoid varnish or lacquer, or other suitable cementing resinoid material in the uncured stage, such as a resinoid powder capable of plastic flow when subjected to heat and pressure. This cement is employed as a thin film between the parts, and this may take the form of a thin paper impregnated with liquid "Bakelite" resinoid in the uncured stage. One or more layers of this impregnated paper 14, which has been cut to the desired annular shape as indicated in Fig. 1, is interposed between the premolded and precured abrasive rim 10 and the annular plane face of the cup 12. Then this assembly of the three parts is compressed in a suitable mold and heat is applied to set the cement.

The mold shown in Fig. 2 may comprise a metal mold band 16 having two metal plates 17 and 18 slidably mounted therein, with a further metal plate 19 fitting the inner portion of the cup. A metal core 20 may be inserted in holes in the metallic parts 17, 18 and 19 as well as the central hole 21 of the cup, so as to prevent deformation of the cup during the pressing operation. The parts will be so sized that the mold plates 17 or 18 will initially project slightly outside of the mold band 16. Then, when the mold with its assembled wheel parts is placed between the two platens of a power press, and pressure is applied to the plates 17 and 18, these plates will be forced towards each other until the mold is closed, or until the press platens rest on the top and bottom plane surfaces of the ring 16.

Prior to this final molding assembly operation, it is feasible to roughen the opposed flat surfaces of the abrasive rim 10 and the top face of the cup 12, such as by means of a grinding wheel or abrasive cloth, so that the cementitious material will make a more intimate contact with each of the opposed bodies. Moreover, it is desirable that the cup 12 be not in a heat set condition so that the roughened surface opposed to the abrasive rim will be capable of flowing slightly into a very intimate union with the resinoid cement and the rim.

Thereafter, the resinoid of the cement and of the backing support 12 are cured by means of heat, in accordance with the standard practice. This may be accomplished by heating the assembled parts of the pressure mold with the wheel enclosed therein and maintaining such temperature conditions as will cause the resinoid to be converted to its final hard infusible condition. Upon disassembling the mold parts, it will now be found that the abrasive rim 10 has been made integral with its backing plate 12.

The same procedure will be in general adopted if a rubber backing plate is to be employed, and in this case a previously compressed and shaped

mass of rubber and sulfur compound which has not been fully vulcanized will be employed for the backing plate. The rubber compound comprises raw rubber, sulfur and a vulcanization accelerator proportioned for making hard rubber, according to standard practice. A rubber cement, with or without a plastic layer of raw rubber compound, or other suitable rubber cementing material, is preferably interposed between this backing cup and the rubber bonded abrasive rim 10. The rubber cementing layer 14 will be provided with sufficient vulcanizing compound, such as sulfur, so that it may be cured to either a resilient or a hard, non-resilient condition as may be desired. Other methods which are standard in the rubber industry may be employed for this procedure.

The following procedure may be adopted if it is desired to make a grinding wheel of the type shown in Fig. 3, which comprises a central supporting disk or cylinder 24 carrying an abrasive rim 25 mounted on its peripheral surface. In this case the abrasive rim 25 may be made as above described of abrasive grains together with a resinoid or rubber bonding compound and these two ingredients may be suitably shaped in a mold having movable parts arranged to provide a cavity of the required dimensions. After the ring 25 is shaped, it may be cured in its original mold or apart therefrom as is desired, so as to form a fully cured body which is to be integrally united with the central support 24. This support will be preferably formed as above described of either a resinoid compound or vulcanizable rubber. These two separately fashioned bodies 24 and 25 may be placed in a mold and there united under heat and pressure.

The pressure mold may comprise a metal band 26 which is L-shaped in cross section so as to provide two inner faces 27 and 28 and an inner shoulder 29. This shoulder 29 is of the exact width of the ring 25, as illustrated in the drawing, so that the premolded and precured ring 25 will be supported wholly on the band 26. A mold plate 30 is slidably mounted within the inner peripheral face 28 of the band, and another press plate 31 slidably fits within the larger peripheral surface 27. If desired, the mold band 26 and the upper plate 31 may be removably secured together by a series of set screws 32 which fit into a groove in the edge of the peripheral face of the plate 30 and thus serve to lock the plate 31 to the mold band 26 during either the pressing or the heating operation.

The central supporting body 24 is preferably slightly oversize in thickness so as to provide material for plastic flow, and if desired an appropriate resinoid or rubber cement 33 as above described may be interposed between this central support and the abrasive rim 25. A metal core 34 is suitably mounted in the central holes in the plates and wheel support 24, so as to support the body 24 against distortion during the pressing operation.

When the mold assembly is pressed between the platens of a power press, the plate 30 will be forced inwardly until the mold is closed and thus will compress only the central supporting mass 24 which is in a slightly plastic condition. This causes a flow of the resinoid material of the support 24 in an outward or a radial direction and thus forces this central mass into a very intimate and complete contact with the matured rim 25. This rim can stand the lateral pressure of the plastic flowing material but it is preferred to

prevent it from being pressed on its top and bottom faces which contact with the plate 31 and the shoulder 29 of the band 26. Hence, the mold is shaped as illustrated and the lock screws 32 are preferably used to prevent an improper application of pressure on the abrasive rim. The central supporting body is comparatively large and so is capable of withstanding the pressure usually employed in a power press, which may be as much as 1 ton per square inch. Also, if the rim lies flat against its support, as shown in Figs. 1 and 2, it may be subjected to the full pressure; whereas pressure should not be applied against the narrow face of the rim when the parts are arranged as shown in Fig. 3.

15 The methods above described may be varied widely within the knowledge of one skilled in the art; but in any case it is desirable that the rim be not only premolded but also heat set prior to its assembly with the central support. Furthermore, the cementing medium employed between the rim and the support may be suitably varied, although it is preferred to have it of the same general class of materials as is used for the abrasive bond. Both forms of rim are to be cemented in place, but the pressure applied to the wheel parts during the assembly molding operation insures a very close union therebetween. This is particularly true if the central body 24 of Fig. 3 is not heat set until after the parts have been 30 united. It will be understood that the sizes of the wheel parts and mold parts will be suitably

chosen for the desired results and particularly where the body 24 is to be made slightly oversize in thickness so that it may flow laterally to the desired extent before the mold is closed.

5

I claim:

1. The method of making a composite abrasive wheel having a central support and an abrasive rim comprising the steps of premolding a heat settable material selected from the class consisting of an unconverted resinoid and a vulcanizable rubber compound, and thereby forming a plastic supporting body having substantially its final volume, separately molding a mixture of abrasive grains and a bond of the type selected for the support to form an abrasive rim, heat setting 15 the rim to its final non-plastic condition, thereafter assembling the central support and rim in a pressure mold with a heat settable cement therebetween, pressing the wheel parts without distorting the rim and causing a plastic flow of 20 the support into a firm union with the rim and heating the wheel to set the unconverted material of the support and cement into a final hard condition.

2. A grinding wheel comprising a thin annular rim of premolded, heat set resinoid and abrasive grains, a premolded support of heat set resinoid and a filler, and an intermediate cementing layer securing the rim to the support which is made of paper impregnated with heat 25 set resinoid.

BAALIS SANFORD.